

Nov. 15, 1949

L. W. DAVIS

2,488,054

PRODUCTION OF MAGNESIUM NITRIDE

Filed April 17, 1945



## UNITED STATES PATENT OFFICE

2,488,054

## PRODUCTION OF MAGNESIUM NITRIDE

Lewis W. Davis, Beverly, Mass., assignor to Metal Hydrides Incorporated, Beverly, Mass., a corporation of Massachusetts

Application April 17, 1945, Serial No. 588,841

9 Claims. (Cl. 23—191)

1

This invention relates to magnesium nitride and has for its object certain improvements in the method of producing magnesium nitride.

It has been proposed to produce magnesium nitride by heating a body of magnesium metal in a stream of nitrogen or ammonia. This method has not achieved any commercial success, largely because the product produced is in fact not magnesium nitride but is a core of magnesium metal with a coating of magnesium nitride. When, for example, magnesium powder or granules or liquid is treated with nitrogen gas in the customary manner, the nitriding reaction takes place only at the surface; so that the theoretical composition of magnesium nitride is not obtained. In other words, what is obtained is partially-nitrided magnesium.

My investigations confirm my discovery that magnesium nitride of high purity, instead of a core of magnesium metal with a coating of magnesium nitride, may be produced, provided the method employed to nitride the magnesium is properly conducted.

In accordance with the invention, magnesium nitride is produced by reacting sublimed magnesium with nitrogen gas at a temperature below that at which the magnesium nitride dissociates but at which the magnesium combines with the nitrogen.

To this end a charge of magnesium metal is heated with applied heat to a temperature sufficiently high to initiate the nitriding reaction and to sublime or vaporize the magnesium. Magnesium tends to sublime below its fusion or melting point, which at normal pressures is 651° C., so that the temperature of the charge is advantageously kept below that temperature. The amount of sublimation is appreciable at temperatures as low as 550° C. A similar effect may, however, be obtained by reacting the vapors of magnesium with nitrogen gas. Since the boiling point of magnesium is 1110° C. at normal pressures, the charge must be considerably raised in temperature to vaporize the magnesium. Since sublimation of the magnesium begins well below the melting or fusion point and continues up to the boiling or vaporizing point of magnesium, the range of sublimation is rather wide, for example from about 550° C. to just below 1110° C. So far as the practice of the invention goes, it is unnecessary to boil the magnesium, although the temperature of the charge may be raised that high, if desired. In any event, the temperature of the charge, and hence of the reaction zone in which the nitriding reaction is conducted, should be be-

2

low the dissociation point of the magnesium nitride, which is 1500° C. at normal pressures.

Since the nitriding reaction is strongly exothermic, the generated heat may be used to carry the reaction to completion. In that case, the use of applied heat may be stopped after the nitriding reaction is given a good start. Depending upon operating conditions, it may be necessary to take special precautions to avoid overheating the charge.

The charge is preferably in the form of relatively small pieces of magnesium metal, such as granules, although other forms may, of course, be employed. The pieces of magnesium are gradually heated to a temperature sufficiently high to cause the nitriding reaction to begin. At this temperature the pieces of magnesium in touch with the nitrogen gas nitride at their surfaces, thus providing a coating or film of magnesium nitride on the pieces of magnesium. While this coating of magnesium nitride forms a barrier to further penetration of the nitrogen gas toward the interior of the pieces of magnesium, it prevents the pieces from sticking to one another or fusing into a solid mass as the temperature of the charge continues to rise.

Instead of stopping at this point, the heating of the partially-nitrided charge of magnesium is continued to effect the sublimation or vaporization of the un-nitrided magnesium in the interior of the coated pieces of magnesium. The sublimed or vaporized magnesium is forced through the coating or film of magnesium nitride at the outside surfaces of the pieces of magnesium and then rises in the reaction zone in contact with the nitrogen gas. Each molecule of sublimed or vaporized magnesium is thus brought into reactive contact with nitrogen and is converted to magnesium nitride. The heating of the original charge of magnesium is continued until all, or substantially all, of the metallic magnesium in the interior of the partially nitrided particles of magnesium, is thus expelled and nitrided.

In a presently preferred practice, a suitable temperature variation is maintained in the reaction zone to effect not only the sublimation or vaporization of the magnesium but to condense the resulting magnesium nitride. To this end, for example, a vertical retort may be employed, the charge of magnesium being placed in the bottom thereof. The highest temperature in the reaction zone is maintained at or near the bottom of the retort, while the upper part of the retort is kept relatively cool. As the sublimed or vaporized magnesium rises upwardly in the re-

action zone from the charge of partially nitrided magnesium and is converted to magnesium nitride, the resulting particles of magnesium nitride tend to condense or settle out at the side wall of the retort, some of the particles, of course, falling down into the charge. After all of the un-nitrided magnesium is expelled from the charge, the residue remaining at the bottom of the retort is, of course, also magnesium nitride. The retort is cooled and opened, after which the magnesium nitride is suitably removed.

To assure high purity magnesium nitride, it is advantageous to confine the charge of magnesium in the retort and to evacuate the reaction zone and charge to remove air and moisture therefrom. Gradually heating the charge to a temperature short of that at which practical sublimation takes place facilitates removal of the air and moisture during the evacuating step. The retort is then filled with a suitable inert gas, such as helium or argon. Enough inert gas is preferably admitted to the retort to place the reaction zone and charge under substantial positive pressure, for example 5 pounds. When, therefore, nitrogen gas or a source of nitrogen gas, such as ammonia, is admitted to the reaction zone, and is consumed by the magnesium, the presence of the inert gas under positive pressure prevents the creation of a vacuum in the retort. While the nitriding reaction may be conducted under vacuum, it is disadvantageous in case the retort should spring a leak. In that case, outside air and moisture would seep into the retort until the vacuum is broken. It is therefore better practice to maintain the reaction zone in the retort under positive pressure with the inert gas, because, in the case of a leak, inert gas would seep out of the retort instead of air seeping into the retort.

In addition, the presence of the inert gas in the retort facilitates temperature control of the nitriding reaction. It serves to dilute the nitrogen gas or ammonia admitted to the reaction zone, thus helping to slow down the nitriding reaction while avoiding the danger of a vacuum being established in case the retort should spring a leak.

While nitrogen gas may be admitted to the reaction zone, ammonia may be similarly admitted as the source of nitrogen gas. At the nitriding reaction, the ammonia is dissociated into nitrogen gas and hydrogen gas, both gases being in nascent form and therefore highly reactive. The hydrogen gas tends to combine with surface oxide on the pieces of magnesium, to form moisture and then steam, and thus cleans or conditions the surfaces for nitriding with the nascent nitrogen. The nascent nitrogen tends also to react more readily with the sublimed or vaporized magnesium than does ordinary nitrogen gas.

These and other features of the invention will be better understood by referring to the accompanying drawing, taken in conjunction with the following description, which illustrates diagrammatically an elevational view, mostly in cross-section, of an apparatus that may be employed in the practice of the invention.

The apparatus shown comprises an outer retort 10 supported within a heating furnace 11, the retort being held in position by means of a plurality of supports 12 spaced under and around a circumferential flange of the retort and resting on the top of the heating furnace. The retort is made preferably of heat-resistant steel. It is provided with a removable cover 13 having attached thereto a vertical pipe 14 with valved

branches 15, 16 and 17 connectible with a source of vacuum, nitrogen gas or ammonia, and inert gas, such as helium or argon, respectively. A gasket 18 is disposed between the cover and the flanged top portion of the outer retort, the three elements forming a non-leakable connection by means of a plurality of spaced bolts 19. A removable inner retort 20 having an open top rests within the outer retort.

The heating furnace consists essentially of a box-like chamber 21 having a refractory bottom 22, side and end walls 23 and a top 24 with an opening of a size adapted to receive the outer retort. An expanding opening 25 is provided at or near a lower corner of one of the side walls of the chamber, for the introduction of heating gases into the chamber. A flue opening 26 extends through another wall, preferably at a higher level, so that heating gases passed into the chamber through opening 25 tend to pass around and in contact with the outer retort before leaving the chamber through the flue opening.

The apparatus may be used as follows:

A charge of magnesium metal, preferably in small or granular pieces, is placed on the bottom of inner retort 20. The retort is then placed in outer retort 10; gasket 18 is placed in position on the circumferential flange of the outer retort; cover 13 is placed thereon; and it is non-leakably secured to the outer retort by bolts 19. In a presently-preferred practice, heating gases are passed through opening 25 into heating chamber 21, while the valve in branch 15 is opened to evacuate air and moisture from the retorts. The heating gases circulate around and in contact with outer retort 10, where they give up a good deal of their heat, after which the spent gases pass through flue opening 26. Heating of the charge in this manner is continued as its temperature rises and reaches a point short of that at which practical sublimation of the magnesium occurs in order to facilitate removal of the air and moisture. The valve in branch 15 is closed when the evacuating step is completed.

The valve in branch 17 is then opened, in a preferred practice, to admit inert gas, such as helium or argon, or both, to the retorts to replace the air evacuated therefrom. A sufficient amount of the inert gas is advantageously passed into the retort to break the vacuum and to place and maintain the reaction zone and charge under substantial positive pressure, for example about 5 pounds. After the desired amount of inert gas has been admitted to the retorts, the valve in branch 17 is closed, or, if a pressure valve is used, it may remain open to assure a constant pressure of inert gas in the retorts.

The valve in branch 16 is then opened to admit a limited amount of nitrogen gas or ammonia, or both, to the retorts as the passage of heating gases through chamber 21 is continued, the heating gases being sufficiently hot gradually to heat the charge of magnesium to its nitriding temperature. When this occurs, the surfaces of the pieces of magnesium in contact with the nitrogen gas are promptly nitrided to form a coating, film or layer of magnesium nitride thereon. The partially nitrided pieces of magnesium are in addition heated to a temperature sufficiently high to distill or vaporize the un-nitrided magnesium in the interior portions of the pieces, so that the sublimed or vaporized magnesium is expelled therefrom. As the sublimed or vaporized magnesium tends to rise in the reaction zone of inner

rétoit 20, it comes in contact with nitrogen gas and promptly reacts therewith to form additional magnesium nitride. This additional magnesium nitride is in extremely finely divided form and tends to deposit or condense along the inner wall of the inner retort, as shown. To facilitate deposition of the magnesium nitride, the inner and outer retorts are provided with a suitable temperature gradient, the hottest portion being at or near the bottom thereof while the cooler portions are at the upper end. This desirable condition is obtained by having the upper portions of the inner and outer retorts extend a suitable distance above heating furnace 11 into the open atmosphere so that heat may be rapidly dissipated therefrom.

As the nitriding action continues, regulated amounts of nitrogen gas or ammonia are admitted to the retorts. Due to the exothermic nature of the nitriding reaction, the amounts thus admitted are regulated in such a manner as to generate heat in amount to maintain the reaction zone at the nitriding temperature but below that at which the magnesium nitride dissociates. Control of the amount of heat generated is also effected in part preferably by regulating the amount of heat dissipated from the reaction zone. This control may be obtained, for example, by using retorts with a predetermined and optimum amount of radiating surface and by placing a charge of magnesium of predetermined and optimum amount in the inner retort. Other means, such as cooling, may be employed to regulate the rate at which heat is dissipated from the retorts. After the nitriding reaction is given a good start initially, the use of applied heat may be stopped; that is, passage of heating gases into chamber 21 may be discontinued. The heat necessary to complete the nitriding operation is then supplied solely by the generated heat. If the temperature of the reaction zone should fall too low, applied heat would, of course, again be used.

In the construction shown, the top portion of inner retort 20 is almost on a level with the upper portion of outer retort 10. This arrangement tends to keep the magnesium nitride within inner retort 20. That is to say, the magnesium nitride formed from the sublimed or vaporized magnesium is condensed or deposited on the inner wall of the inner retort before it has a chance to rise above the top portion of the inner retort.

As pointed out above, if ammonia is used as the source of hydrogen gas, on admission to the retorts, it is heated to a temperature sufficiently high to dissociate it into nascent nitrogen gas and nascent hydrogen gas. The nascent hydrogen tends to react with surface magnesium oxide, if present, on the pieces of magnesium metal in the charge, to form moisture which, at the elevated temperatures employed, is promptly converted into steam. The nascent nitrogen then reacts with the cleansed metallic surfaces on the pieces of magnesium metal to form a coating, film or layer of magnesium nitride. The nascent nitrogen appears to be more highly reactive than ordinary nitrogen gas as a nitriding agent.

When all of the metallic magnesium in the interior portions of the partially nitrided pieces of magnesium in the charge has been sublimed or volatilized, and the nitriding reaction has gone to completion, the retorts and their contents are permitted to cool. Cover 13 is then removed from outer retort 10, inner retort 20 is removed from the outer retort 10, and the magnesium nitride is

scraped or otherwise removed from the inner retort.

The operation described results in a substantially complete conversion of all of the available magnesium in the charge to magnesium nitride, the efficiency of the nitriding reaction being exceedingly high, so that a product of high purity is obtained. The purer the magnesium placed in the inner retort, the purer will be the magnesium nitride produced by the nitriding operation. Since the metallic magnesium in the interior portions of the pieces of magnesium metal is expelled into an atmosphere of nitrogen, complete nitridation of all of the magnesium metal is assured.

It will be clear that the above example is only by way of illustration, and that various modifications thereof may be employed in the practice of the invention. For convenience, the magnesium expelled from the pieces of partially nitrided magnesium is referred to in the claims as sublimed magnesium, although this terminology is intended also to include vaporized or distilled magnesium.

I claim:

1. In the method of producing magnesium nitride, the improvement which comprises confining a charge consisting of a plurality of pieces of magnesium metal in a reaction zone, admitting a limited amount of nitrogen to the reaction zone, gradually heating the charge to a temperature sufficiently high to cause the nitrogen to react with the pieces of magnesium at their surfaces to form a coating of magnesium nitride thereon, gradually heating the partially nitrided charge to a temperature sufficiently high to sublime magnesium from the interior portions of the coated pieces of magnesium and to make the sublimed magnesium break through the surface coating of magnesium nitride on the pieces of magnesium, gradually admitting additional amounts of nitrogen to the reaction zone, and converting the sublimed magnesium as it rises in the reaction zone to magnesium nitride with the nitrogen.

2. In the method of producing magnesium nitride, the improvement which comprises confining a charge consisting of a plurality of pieces of magnesium metal in a reaction zone, evacuating the reaction zone to remove air and moisture therefrom, admitting a limited amount of nitrogen to the reaction zone, gradually heating the charge to a temperature sufficiently high to cause the nitrogen to react with the pieces of magnesium at their surfaces to form a coating of magnesium nitride thereon, gradually heating the partially nitrided charge to a temperature sufficiently high to sublime magnesium from the interior portions of the coated pieces of magnesium and to make the sublimed magnesium break through the surface coating of magnesium nitride on the pieces of magnesium, gradually admitting additional amounts of nitrogen to the reaction zone, and converting the sublimed magnesium as it rises in the reaction zone to magnesium nitride with the nitrogen.

3. In the method of producing magnesium nitride, the improvement which comprises confining a charge consisting of a plurality of pieces of magnesium metal in a reaction zone, evacuating the reaction zone to remove air and moisture therefrom, admitting inert gas to the reaction zone in amount sufficient to place and maintain it and the charge under substantial positive pressure, admitting a limited amount of nitrogen to the reaction zone, gradually heating the charge

to a temperature sufficiently high to cause the nitrogen to react with the pieces of magnesium at their surfaces to form a coating of magnesium nitride thereon, gradually heating the partially nitrided charge to a temperature sufficiently high to sublime magnesium from the interior portions of the coated pieces of magnesium and to make the sublimed magnesium break through the surface coating of magnesium nitride on the pieces of magnesium, gradually admitting additional amounts of nitrogen to the reaction zone, and converting the sublimed magnesium as it rises in the reaction zone to magnesium nitride with the nitrogen.

4. In the method of producing magnesium nitride, the improvement which comprises confining a charge consisting of a plurality of pieces of magnesium metal in a reaction zone, evacuating the reaction zone to remove air and moisture therefrom, admitting a limited amount of nitrogen to the reaction zone, gradually heating the charge to a temperature sufficiently high to cause the nitrogen to react with the pieces of magnesium at their surfaces to form a coating of magnesium nitride thereon, gradually heating the partially nitrided charge to a temperature sufficiently high to sublime magnesium from the interior portions of the coated pieces of magnesium and to make the sublimed magnesium break through the surface coating of magnesium nitride on the pieces of magnesium, gradually admitting additional amounts of nitrogen to the reaction zone, converting the sublimed magnesium as it rises in the reaction zone to magnesium nitride with the nitrogen, and regulating the amounts of nitrogen thus admitted to the reaction zone to an amount insufficient on combining with the sublimed magnesium to generate sufficient heat to decompose the magnesium nitride.

5. In the method of producing magnesium nitride, the improvement which comprises confining a charge consisting of a plurality of pieces of magnesium metal in a reaction zone, admitting a limited amount of nitrogen to the reaction zone, gradually heating the charge with applied heat to a temperature sufficiently high to cause the nitrogen to react with the pieces of magnesium at their surfaces to form a coating of magnesium nitride thereon, gradually heating the partially nitrided charge to a temperature sufficiently high to sublime magnesium from the interior portions of the coated pieces of magnesium and to make the sublimed magnesium break through the surface coating of magnesium nitride on the pieces of magnesium, terminating the use of applied heat, gradually admitting additional amounts of nitrogen to the reaction zone, converting the sublimed magnesium as it rises in the reaction zone to magnesium nitride with the nitrogen, and regulating the rate of nitrogen thus admitted to the reaction zone to an amount which on combining with the sublimed magnesium generates heat insufficient in amount to decompose the magnesium nitride but sufficient in amount to carry the nitriding operation to completion.

6. In the method of producing magnesium nitride, the improvement which comprises confining a charge consisting of a plurality of pieces of magnesium metal in a reaction zone, evacuating the reaction zone to remove air and moisture therefrom, admitting inert gas to the reaction zone in amount sufficient to place and maintain it and the charge under substantial positive pressure, admitting a limited amount of nitrogen to

the reaction zone, gradually heating the charge with applied heat to a temperature sufficiently high to cause the nitrogen to react with the pieces of magnesium at their surfaces to form a coating of magnesium nitride thereon, gradually heating the partially nitrided charge to a temperature sufficiently high to sublime magnesium from the interior portions of the coated pieces of magnesium and to make the sublimed magnesium break through the surface coating of magnesium nitride on the pieces of magnesium, terminating the use of applied heat, gradually admitting additional amounts of nitrogen to the reaction zone, converting the sublimed magnesium as it rises in the reaction zone to magnesium nitride with the nitrogen, and regulating the rate of nitrogen thus admitted to the reaction zone to an amount which on combining with the sublimed magnesium generates heat insufficient in amount to decompose the magnesium nitride but sufficient in amount to carry the nitriding operation to completion.

7. In the method of producing magnesium nitride, the improvement which comprises placing a charge of magnesium in a confined reaction zone, evacuating the reaction zone to remove air and moisture therefrom, heating the reaction zone to maintain the magnesium above its sublimation temperature but below its boiling temperature, admitting a limited amount of a gas selected from the group consisting of nitrogen and ammonia to the reaction zone to initiate the nitriding reaction and limit the exothermic heat generated by the reaction to an amount insufficient to raise the temperature of the reaction zone above said boiling temperature, reacting nitrogen with the charge of magnesium at its surface to form a coating of magnesium nitride thereon, heating the partially nitrided charge to a temperature sufficiently high to cause sublimed magnesium to break through the surface coating of magnesium nitride on the charge and to cause the sublimed magnesium as it moves away from the charge to react with nitrogen to form magnesium nitride, gradually admitting further amounts of said gas to the reaction zone to continue the nitriding reaction, and regulating the rate of formation of the magnesium nitride and hence the rate of generation of exothermic heat by controlling the rate at which said further amounts of said gas are admitted and thereby maintain the temperature of the reaction zone below said boiling temperature.

8. In the method of producing magnesium nitride, the improvement which comprises confining a charge of magnesium metal in a reaction zone, admitting a limited amount of nitrogen to the reaction zone, gradually heating the charge to a temperature sufficiently high to cause the nitrogen to react with the charge of magnesium at its surface to form a coating of magnesium nitride thereon, gradually heating the partially nitrided charge to a temperature sufficiently high to sublime magnesium from the interior portion of the coated charge of magnesium and to make the sublimed magnesium break through the surface coating of magnesium nitride on the charge of magnesium, gradually admitting additional amounts of nitrogen to the reaction zone, and converting the sublimed magnesium as it rises in the reaction zone to magnesium nitride with the nitrogen.

9. In the method of producing magnesium nitride, the improvement which comprises con-

fining a charge of magnesium metal in a reaction zone, evacuating the reaction zone to remove air and moisture therefrom, admitting inert gas to the reaction zone in amount sufficient to place and maintain it and the charge under substantial positive pressure, admitting a limited amount of nitrogen to the reaction zone, gradually heating the charge to a temperature sufficiently high to cause the nitrogen to react with the charge of magnesium at its surface to form a coating of magnesium nitride thereon, gradually heating the partially nitrided charge to a temperature sufficiently high to sublime magnesium from the interior portion of the charge of magnesium and to make the sublimed magnesium break through the surface coating of magnesium on the charge of magnesium, gradually admitting additional amounts of nitrogen to the reaction zone, and converting the sublimed magnesium as it rises in the reaction zone to magnesium nitride with the nitrogen.

LEWIS W. DAVIS.

#### REFERENCES CITED

The following references are of record in the file of this patent:

#### UNITED STATES PATENTS

| Number    | Name  | Date          |
|-----------|-------|---------------|
| 1,319,843 | Burke | Oct. 28, 1919 |
| 1,803,720 | Miner | May 5, 1931   |

#### OTHER REFERENCES

Maxted, "Ammonia And The Nitrides," 1921 ed., J. & A. Churchill, London, publishers, pages 49, 54-56 and 67-68.

15 Mellor's "Modern Inorganic Chemistry," 1939 ed., Longmans, Green & Co., N. Y., publishers, pages 385 and 386.

15 Mellor, "A Comprehensive Treatise on Inorganic and Theoretical Chemistry," 1928 ed., vol. VIII, Longmans, Green & Co., N. Y., publishers, 20 page 104.

**Certificate of Correction**

Patent No. 2,488,054

November 15, 1949

LEWIS W. DAVIS

It is hereby certified that errors appear in the printed specification of the above numbered patent requiring correction as follows:

Column 1, line 4, and lines 25 and 26, for "megnesium" read *magnesium*; column 4, line 42, for "sublimination" read *sublimation*; column 10, list of references cited, line 16, for "pages 385 and 386" read *pages 622 and 623*;

and that the said Letters Patent should be read with these corrections therein that the same may conform to the record of the case in the Patent Office.

Signed and sealed this 7th day of March, A. D. 1950.

**[SEAL]**

THOMAS F. MURPHY,  
*Assistant Commissioner of Patents.*